

## 1

3,356,471

## TRIARYL PHOSPHATE MIXTURES

Edmund L. Niedzielski, Wilmington, Del., assignor to  
E. I. du Pont de Nemours and Company, Wilmington,  
Del., a corporation of Delaware  
No Drawing. Filed Aug. 9, 1963, Ser. No. 301,183  
15 Claims. (Cl. 44—69)

This invention relates to novel mixtures of aryl triesters of orthophosphoric acid and to compositions containing them.

The art, as reviewed for example by Popkin in U.S. Patent 3,034,877, is well aware of the problems associated with the use of organolead compounds as antiknock agents in gasoline. In combating these problems, the art has generally resorted to the joint use of one or more halohydrocarbons, particularly ethylene dibromide and ethylene dichloride as first proposed by Midgely in U.S. Patent 1,668,022 and further amplified by Bartholomew in U.S. Patent 2,398,281, which function to scavenge lead through the formation of divalent lead halides. Thus, lead, which otherwise would remain deposited in the combustion zone as oxidized lead, such as the oxide, oxyhalide and sulfate, may be exhausted from the engine in the form of relatively volatile dihalides. However, the halogen compounds are incompletely effective and the engine gradually accumulates deposits which contribute to such undesirable conditions as increase in the octane requirement of the engine, spark plug fouling by decreasing the electrical resistance of plug insulation, and untimely ignitions by inducing the fuel-air charge to fire before normal spark ignition can take place. The problem of preignition (also referred to as surface ignition) is particularly serious in high compression spark ignition engines. Erratic ignitions lead to rough engine operation, reduced power output, increased wear and erosion of engine parts.

The art has also long been aware that compounds of phosphorus are sometimes beneficial to inhibit spark plug misfiring, to suppress deposit-induced preignitions and to assist the normally employed halohydrocarbon additives in removing combustion chamber deposits. Popkin, in U.S. Patent 3,034,877, proposes to use monoalkyl diphenyl phosphates to solve some of these problems.

Fry et al., in U.S. Patent 2,375,218, disclose treating spark plug porcelains with a phosphorus compound, then heating to a high temperature to promote the desired reaction of the phosphorus compound with the deposits in or on the spark plug enamel. When the phosphorus compound is to be carried in a leaded gasoline, trimethyl phosphate is recommended since other phosphorus compounds are said to depreciate the antiknock value of the tetraethyl lead.

Livingston, in an article "Antiknock Antagonists," Industrial and Engineering Chemistry, 43, pp. 663-670 (1951), reports that tetraethyl lead is extremely sensitive to the antagonism of phosphorus and its compounds.

In view thereof, British Patent 683,405 proposes the use of completely esterified organic esters of phosphorus (or arsenic) containing at least one carbocyclic radical. Tricresyl phosphate, triphenyl phosphate, 2-naphthyl diphenyl phosphate and trinaphthyl phosphate, among others, are disclosed to be effective, individually, to offset the tendency of the octane requirement of the engine to increase with use, reduce exhaust valve corrosion, and counteract spark plug fouling, without adversely affecting fuel antiknock quality.

Yust and Bame, in U.S. Patent 2,889,212, which is apparently based on British Patent 683,405, disclose that the joint use of a halohydrocarbon scavenger and an alkaryl phosphate (or phosphite), e.g., tricresyl phosphate, substantially eliminates spark plug fouling without deleteriously affecting the antiknock characteristics of the fuel.

## 2

It appears that the alkaryl phosphate-halohydrocarbon scavenger compositions are especially designed for use in aviation fuels because of the relatively more frequent occurrences of spark plug fouling and the severity of the problem in aviation engines. In other words, the alkaryl phosphate-based compositions are selected primarily for their effectiveness as spark plug antifoulants on the basis of tests conducted with aviation grade gasolines. It appears that the presence of at least one alkaryl radical in the phosphorus compound is essential for good spark plug antifouling activity, as triphenyl phosphate is shown to be much less effective than tricresyl phosphate.

Aviation grade gasolines, as a rule, are especially olefin-free and contain not more than about 5 volume percent of aromatic hydrocarbons. In recent years, motor fuels have been developed which contain substantial amounts of aromatics, first proposed by Wagner et al. in "Improved Motor Fuels Through Selective Blending," paper presented before 22nd Meeting of the American Petroleum Institute, Nov. 7, 1941. The aromatic components constitute heavy-ends, i.e., high-boiling fractions of such gasolines, and these high aromatic content heavy-ends have been found more prone to produce deposits which cause surface ignition than other gasoline hydrocarbon types. Since, in multicylinder engines, fractionation of the fuel occurs during certain phases of engine operation, with light-end and heavy-end components being unevenly distributed to the various cylinders, the surface ignition problem tends to be further aggravated in cylinders getting a greater than normal share of aromatic components.

Thus, it is particularly desirable to be able to provide an effective means of controlling surface ignitions in modern high compression ratio spark ignition engines operating on high aromatic content motor gasolines.

While the art recognizes that one or more of such diverse problems as spark plug fouling, surface ignition, octane requirement increase, and exhaust valve corrosion may be attributed largely to the accumulation of combustion chamber deposits and may in part be alleviated through use of fuel additives, it has become keenly aware that more often an additive effective in one regard is disappointing in another. Thus, Gilbert, in U.S. Patent 2,897,071, points out that "the alleviation of spark plug failure is generally attained at the expense of both exhaust valve life and destructiveness of the organolead antiknock agent," and further states: "Regarding many of the problems frequently associated with high octane quality fuel, an anomalous situation obtains. On one hand an effective adjuvant for organolead compounds should possess stability against deterioration in common environments, compatibility with the chemical entities with which it comes in contact, and volatility so as to possess the characteristic frequently referred to as engine inductibility. On the other hand, the mere selection of a phosphorus compound to acquire the optimum characteristics enumerated above does not necessarily assure the effectiveness of the compound in combating such phenomena as spark plug fouling, wild ping and the like. It is entirely probable that some empirical relationship between physical properties and effectiveness in the obviation of such problems exists, but as yet the state of the art does not contain a satisfactory relationship of this type."

It is an object of this invention to provide improved combustion chamber deposit scavenging compositions for use in leaded motor fuels, particularly those high in aromatic hydrocarbons. Another object is to provide novel triaryl phosphate compositions which are particularly effective, in conjunction with halohydrocarbon scavengers in leaded high octane number high aromatic content motor gasolines, to suppress surface ignition and combat spark plug fouling, and which tend to minimize the octane

number requirement of the engine and reduce exhaust valve corrosion, substantially without adverse effect on the antiknock quality of the gasoline. Still another object is to provide such compositions which provide the further benefit of imparting significant anti-stall properties to motor gasolines at the same concentrations that are useful for attaining the above objects concerning combustion chamber performance. A further object is to provide new motor fuels comprised essentially of high octane number high aromatic content base gasolines, organolead antiknock agents, halohydrocarbon scavengers for lead, and novel triaryl phosphate compositions, to provide improved combustion chamber performance. A still further object is to provide such new motor gasoline compositions which show improved performance during the induction phase of engine operation as well as during the combustion phase. Other objects are to provide new compositions of matter and to advance the art. Still other objects will appear hereinafter.

The above and other objects are achieved according to this invention by employing, in aromatic motor fuels, organolead antiknock agents and halohydrocarbon lead scavengers in combination with novel triaryl phosphate compositions consisting essentially of

- (a) about 20 to about 50 mole percent of triphenyl phosphate,
- (b) about 35 to about 60 mole percent of a two-ring-aryl diphenyl phosphate,
- (c) about 10 to about 30 mole percent of a di(two-ring-aryl) phenyl phosphate, and
- (d) 0 to about 6 mole percent of a tri(two-ring-aryl) phosphate,
- (e) the mixed phosphates of (b) and (c) constituting a total of about 50 to about 80 mole percent of said mixture, and
- (f) phenyl groups constituting about 60 to about 80 mole percent of all aryl groups in said phosphates.

Said novel triaryl phosphate compositions and antiknock compositions consisting essentially of organolead antiknock agents, with or without halohydrocarbon scavengers for lead, and said triaryl phosphate compositions also constitute important new compositions of this invention.

In the term "two-ring-aryl" as employed herein, "aryl" is used in the strict sense to mean an unsubstituted aromatic hydrocarbon radical, i.e., one which does not contain any alkyl or other substituent on the hydrocarbon rings. Thus, the "two-ring-aryl" radicals consist of naphthyl and biphenyl radicals. Also, "phosphate" means ester of orthophosphoric acid.

The phenyl two-ring-aryl phosphate compositions of this invention are characterized by their many beneficial properties bearing on utility. They are liquid at normal room temperatures (about 25° C.), miscible with the halohydrocarbon scavenger and organolead anti-knock components, and readily soluble in liquid hydrocarbons of the gasoline boiling range. Substantially insoluble in water, they are not extracted from the motor fuel compositions, e.g., when stored over refinery water bottoms. They have not been found to be in any way harmful to the organolead antiknock blends or to the leaded motor fuel compositions. They are cleanly inductible with gasoline and impart significant antistalling properties thereto under conditions normally conducive to carburetor icing. As combustion chamber deposit modifiers, they are particularly effective to combat spark plug fouling and abnormal surface ignition phenomena. At the same time, they tend to reduce the weight of combustion chamber deposits, lower engine octane requirement, and decrease exhaust valve corrosion.

Essentially, the triaryl phosphate compositions of this invention are mixtures of (a) about 20 to about 50 mole percent of triphenyl phosphate, (b) about 35 to about 60 mole percent of a two-ring-aryl diphenyl phosphate, and

(c) about 10 to about 30 mole percent of a di(two-ring-aryl) phenyl phosphate, wherein the mixed phosphates, (b) and (c) constitute a total of about 50 to about 80 mole percent of the mixture and the total of the phenyl groups in the mixture constitute about 60 to about 80 mole percent of all aryl groups present in the mixture of phosphates. Normally, also, the two-ring-aryl diphenyl phosphate will be present in larger proportions than the di(two-ring-aryl) phenyl phosphate. The rather non-volatile tri(two-ring-aryl) phosphates, i.e., the trinaphthyl phosphates and the tribiphenyl phosphates, are not essential components of the tri-aryl phosphate compositions of this invention and, most preferably, should be absent. However, it is not always economically practical to completely eliminate them from the compositions, and they may be tolerated in the compositions in proportions of up to about 6 mole percent, preferably not more than about 4 mole percent.

Preferably, the triaryl phosphate composition will consist essentially of (a) about 25 to about 45 mole percent triphenyl phosphate, (b) about 40 to about 55 mole percent two-ring-aryl diphenyl phosphate, (c) about 15 to about 25 mole percent di(two-ring-aryl) phenyl phosphate, and (d) 0 to about 4 mole percent tri(two-ring-aryl) phosphate, the mixed phosphates of (b) and (c) constituting a total of about 55 to about 75 mole percent of said mixture and the phenyl groups constituting about 65 to about 75 mole percent of all aryl groups in said phosphates. A particularly preferred composition and distribution per mole is about 28 to about 32% triphenyl phosphate, about 44 to about 48% naphthyl diphenyl phosphate, about 20 to about 24% dinaphthyl phenyl phosphate, and 0 to about 4% trinaphthyl phosphate. Another particularly preferred composition and distribution per mole is about 29 to about 33% triphenyl phosphate, about 51 to about 55% biphenyl diphenyl phosphate, about 12 to about 16% di-biphenyl phenyl phosphate, and 0 to about 4% tri-biphenyl phosphate. Mixtures of these compositions may be used. The naphthyl radicals in the compositions may be 1-naphthyl or 2-naphthyl or both, but preferably will be 2-naphthyl. The biphenyl radicals may be one or more of 2-biphenyl, 3-biphenyl or 4-biphenyl, but preferably will be 2-biphenyl radicals.

The triaryl phosphate compositions of this invention are conveniently characterized in terms of the ratio of the phenyl radicals to the total aryl radicals, including phenyl radicals (which ratio multiplied by 100=mole percent phenyl). This ratio or phenyl radical content is directly related to the average molecular weight and the phosphorus content of the composition. Thus, the phosphate compositions of this invention which correspond to phenyl naphthyl triesters containing 80 to 60 mole percent phenyl radicals have average molecular weights ranging from about 355 (8.7% wt. P) to about 385 (8.1% wt. P). Similarly, those corresponding to 80 to 60 mole percent phenyl radicals and 20 to 40 mole percent biphenyl radicals as said triesters have average molecular weights ranging from about 372 (8.3% wt. P) to about 417 (7.4% wt. P). All these compositions are also characterized by their wide boiling range, at least about 95 mole percent boiling over the range of about 225° C. to 350° C. at 5 mm. of Hg pressure.

The multi-component nature of these phosphate compositions is an important feature of the invention. Such compositions are surprisingly fluid compared to the individual components and show good fuel-induction characteristics. Their wide over-all boiling range, together with their good inductibility, may explain to some extent their over-all superior performance in the various critical zones of the combustion chamber, i.e., the exhaust valve region, the walls of the chamber and the spark plug area. Surprisingly, the multicomponent phosphate compositions of this invention are more effective than such commercially employed prior art alkaryl phosphate additives as

tricresyl phosphate and cresyl diphenyl phosphate in controlling surface ignition, and are at least as effective as spark plug antifoulants despite their lower volatility per mole and total lack of alkaryl groups.

The triaryl phosphate compositions of this invention may be prepared by combining the individual components or mixtures thereof, in the designated proportions, said phosphates being obtainable in substantially pure condition by known methods of preparation and purification. Conveniently, the compositions are prepared directly starting with mixtures of phenyl and naphthyl or biphenyl radical sources which are converted to mixed phosphate esters in accordance with known techniques and procedures. For example, mixtures of phenol with beta-naphthol and/or with ortho-phenylphenol are reacted with phosphorus oxychloride in the presence of a catalyst such as  $AlCl_3$  or  $MgCl_2$  to produce mixed triesters of orthophosphoric acid. Normally, mixtures, consisting of from 1.5 to 4 moles of the phenol, preferably 2 to 3 moles, for each mole of the naphthol or phenylphenol, are reacted with an equimolar proportion of phosphorus oxychloride and the catalyst in an amount of from 0.25-1% by weight of the charge at elevated temperatures (initially at 80° C.-110° C. and finally at 170° C.-190° C.) until the evolution of the hydrogen chloride by-product is complete. The composition of the resulting product mixture is readily determined by known methods of analysis. Phenol: naphthol or phenylphenol mole ratios of 1.5-4:1 normally produce mixtures consisting broadly per mole of 20-50% triphenyl phosphate, 35-50% two-ring-aryl diphenyl phosphate, 10-30% di(two-ring-aryl) phenyl phosphate, and from essentially nil (less than 1.0%) to 6% tri(two-ring-aryl) phosphate. Preferred ratios of 2-3:1 yield mixtures composed of 25-45% triphenyl phosphate, 40-50% two-ring-aryl diphenyl phosphate, 12 to 25% di(two-ring-aryl) phenyl phosphate, and up to 3% tri(two-ring-aryl) phosphate.

Normally, the product mixtures of the above process are washed acid-free with dilute alkali and water, and may be used in such form directly in accordance with this invention. If desired, the product may be distilled either for purposes of further purification, or to obtain one or more of the individual components in the substantially pure state, or to alter the composition, e.g. by removing part of the triphenyl phosphate fraction or by distilling away the triphenyl and the unsymmetrical two-ring-aryl phenyl phosphates from the higher boiling tri(two-ring-aryl) phosphate component.

The triaryl phosphate compositions of this invention will be used in conjunction with an organolead anti-knock agent in amounts providing about 0.013 to about 0.4 atom of phosphorus per atom of lead of the organolead anti-knock agent, preferably about 0.033 to about 0.27 atom of phosphorus per atom of lead. These amounts, based on the formation of  $Pb_2(PO_4)_3$ , correspond to about 0.02 to about 0.6 theory of phosphorus, preferably about 0.05 to about 0.4 theory.

The organolead antiknock agent may be any of those known to the art for such purpose, but usually will be a lower ( $C_1-C_4$ ) tetraalkyl lead, such as tetramethyl lead, tetraethyl lead, methyl triethyl lead, dimethyl diethyl lead, trimethyl ethyl lead, tetraisopropyl lead, and the like, and mixtures of any two or more of such organolead anti-knock agents, employed in an antiknock quantity, i.e. in an amount providing 0.1 to 6 grams of lead for each gallon of the motor fuel, preferably about 2 to 4 grams Pb/gal. Preferably, the antiknock agent will be one or more tetraalkyl lead compounds in which the alkyl groups contain 1-2 carbon atoms.

Also, the triaryl phosphate compositions will ordinarily be employed in conjunction with one or more halohydrocarbon scavengers for said lead, but may be used without such scavengers. Such halogen source is believed not critical, on the basis for example that the phosphates of this invention have been found to effect substantially the

same percent reduction in the incidence of surface ignition whether in the absence or in the presence of halohydrocarbon scavengers. Better overall performance has been obtained however with halohydrocarbon scavengers present.

The halohydrocarbon scavenger may be any of those known to the art for use in conjunction with organolead antiknock agents, particularly the halogenated aliphatic, cycloaliphatic and aromatic hydrocarbons wherein the halogens are of atomic numbers 17-35 and which contain 2 to 3 bromo and/or chloro substituents and from 2 to 8 carbon atoms and normally boil below about 250° C. Usually preferred for this use however are the ethylene dihalides—the dibromide, the dichloride, and the chlorobromide—singly or as mixtures of two or more thereof. Normally, also, the quantity of halohydrocarbon scavenger corresponds to from 1-5 atoms (0.5-2.5 theories) preferably about 2 to about 3 atoms (about 1 to about 1.5 theories) of halogen (Cl and/or Br) per atom of lead of the organolead antiknock, and not more than 2 atoms of bromine for each atom of lead. Preferably, for motor fuel use, the quantity of bromine will not exceed about 1 atom of Br per atom of Pb, in other words, not exceed about 0.5 theory, the rest being chlorine.

The triaryl phosphate composition, halohydrocarbon scavenger, and organolead antiknock component may be premixed in any order and in any combination with one another to form antiknock blends for addition to the base fuel. Such blends may also contain other additives normally employed in their formulation, such as identifying dyes, neutral solvent oils (kerosene, toluene, xylene), and gasoline antioxidants. Of course, each additive may be added separately to the fuel or the phosphate composition itself may be added to preexisting leaded motor gasolines to produce the novel improved fuels of this invention.

The mixture of hydrocarbons which constitute the principal component of the fuel compositions of this invention may be a commercial gasoline containing the aromatic hydrocarbons in the defined amounts or it may be a blend of hydrocarbons of the character of those present in such gasolines. Thus, for example, it may be a catalytic-cracked stock, a catalytic-reformed stock, or blends of one or more of these cracked and reformed stocks, or blends of one or more of the above stocks with saturated stocks such as the synthetic alkylates and straight run stocks. Typical aromatic hydrocarbons, which are essential components of the motor fuels of this invention and which are of the character of those aromatic hydrocarbons which are produced in catalytic cracking and catalytic reforming operations, are the mono- and poly-lower alkyl benzenes such as toluene, ethylbenzene, the xylenes, and the like. Typical catalytic-cracked refining stocks contain from about 6 to about 25 volume percent aromatic hydrocarbons, about 29-44 volume percent olefins, the rest saturated hydrocarbons. Catalytic-reformed stocks run higher in aromatics, usually about 40-70 volume percent, and are lower in olefins. Synthetic alkylates are essentially saturated hydrocarbons, high in isoparaffins. Stocks such as these are blended in various proportions for the production of commercial fuels for spark ignition engines. These fuels normally boil within the range of about 80° F. to about 440° F. Blended fuels for commercial use, such as those for automotive use, contain on the average up to about 55 volume percent aromatic hydrocarbons, up to about 30 volume percent olefinic hydrocarbons, the rest saturated hydrocarbons.

The motor fuels of the present invention contain at least 15 volume percent, more usually at least 20 volume percent and not more than about 75 volume percent, aromatic hydrocarbons. Olefinic hydrocarbons are not essential and may be present in the normally occurring proportions. Preferred fuels contain at least about 25 volume percent aromatics and less than 30 volume percent olefins, and have a knock rating of at least 80 as measured

by the ASTM Research Method, most preferably a knock rating of 85 or better. The fuels may also contain other additives normally associated with finished gasolines, such as antioxidants, metal deactivators, dyes, detergents, and antiicing agents.

In order to more clearly illustrate this invention, preferred compositions and modes of practicing it and the advantageous results to be obtained thereby, the following examples are given in which the parts and proportions are by weight except where specifically indicated otherwise.

*Example 1*

A. A mixture, consisting of 11.75 lbs. of beta-naphthol (0.0816 lb. mole), 15.35 lbs. of phenol (0.1632 lb. mole), 12.56 lbs. of phosphorus oxychloride (0.0820 mole) and 0.18 lb. of anhydrous magnesium chloride, is heated in a 10 gallon glass-lined kettle equipped with an agitator and a reflux condenser at temperatures of from 80° C. to 110° C. for 16 hours, during which time HCl is expelled from the reaction mass. The charge is heated to 170° C. to complete the reaction, cooled, washed acid-free in turn with water, dilute aqueous caustic at pH 10, again with water, and dried by heating at 110° C. under reduced pressure to yield 29.35 lbs. of a fluid (at normal room temperatures) mixture of phenyl naphthyl phosphates having high solubility in hydrocarbon solvents and having the properties shown hereinafter in Table 1. The great bulk of the product (94.2% by weight) comprises triphenyl phosphate, naphthyl diphenyl phosphate, and dinaphthyl phenyl phosphate distilling at from about 160° C. to about 265° C. at 0.2 mm. of Hg pressure, with the rest (5.8% weight) being still higher boiling and comprising mainly trinaphthyl phosphate.

Analysis by distillation indicated the composition to be 29 mole percent triphenyl phosphate, 45 mole percent 2-naphthyl diphenyl phosphate, 23 mole percent bis(2-naphthyl)-phenyl phosphate, and 3 mole percent tris(2-naphthyl) phosphate, which corresponds to a phenyl con-

This product, which has a phenyl content of 33% and is thus outside the scope of this invention, will be referred to hereinafter as "PN 33."

*Example 2*

Mixed 4-biphenyl phenyl phosphates were prepared by the procedure of Example 1 from 170 parts 4-hydroxybiphenyl (1 mole), 188 parts phenol (2 moles), 154 parts  $\text{POCl}_3$  (1 mole) and 3 parts anhydrous  $\text{MgCl}_2$ , by heating the mixture for 4 hours between 80° C. and 110° C., and then 8 hours at 180° C. The reaction mass was washed and dried as in Example 1 to yield a fluid (at normal room temperatures), motor gasoline-soluble product having other properties as given in Table 1 and having an overall composition of about 30 mole percent triphenyl phosphate, 51 mole percent 4-biphenyl diphenyl phosphate, 18 mole percent bis(4-biphenyl) phenyl phosphate and 1 mole percent tris(4-biphenyl) phenyl phosphate. The product is referred to hereinafter as "P4-B 70."

*Example 3*

Mixed 2-biphenyl phenyl phosphates were prepared by the procedure of Example 2 except that 2-hydroxybiphenyl (1 mole) was used in place of the 4-hydroxy isomer. Washing and drying the reaction mass as in Example 1 yielded a fluid (at normal room temperatures), motor gasoline-soluble product having a phosphorus content of 7.8% by weight, in substantial agreement with the expected value. 96.2 percent of the product mixture distilled over the range 187° C. to 267° C. at 0.7 mm. of Hg pressure (or at 228° C. to 330° C. at 5 mm. of Hg pressure) to yield a distilled liquid mixture composed of 31 mole percent triphenyl phosphate, 55 mole percent 2-biphenyl diphenyl phosphate, and 14 mole percent bis(2-biphenyl) phenyl phosphate, which corresponds to a phenyl content of 72%. This product mixture will be referred to hereinafter as "P2-B 72."

TABLE 1.—SUMMARY OF PHYSICAL PROPERTIES OF TRIARYL PHOSPHATES  
[Individual components and mixtures of Examples 1-3]

| Phosphate                                                                                         | Physical State <sup>1</sup>      | Boiling Range <sup>2</sup> | Pour Point, ° F. | Viscosity, Centistokes at— |        |
|---------------------------------------------------------------------------------------------------|----------------------------------|----------------------------|------------------|----------------------------|--------|
|                                                                                                   |                                  |                            |                  | 99° C.                     | 38° C. |
| $(\text{C}_6\text{H}_5\text{O})_3\text{PO}$                                                       | Solid, M.P. 50° C. <sup>3</sup>  | 245-250° C./5 mm.          | —                | —                          | (*)    |
| $(\text{C}_6\text{H}_5\text{O})_2(2\text{-C}_6\text{H}_5\text{O})\text{PO}$                       | Liquid <sup>4</sup>              | 285-290° C./5 mm.          | 0                | 5.2                        | 67     |
| $(\text{C}_6\text{H}_5\text{O})_2(2\text{-C}_6\text{H}_5\text{O})\text{PO}$                       | do                               | 330-340° C./5 mm.          | 35               | —                          | 399    |
| $(2\text{-C}_6\text{H}_5\text{O})_3\text{PO}$                                                     | Solid, M.P. 110° C. <sup>4</sup> | —                          | —                | (*)                        | (*)    |
| "PN 67" of Example 1                                                                              | Liquid                           | 225-340° C./5 mm.          | 0                | 5.6                        | 52     |
| $(\text{C}_6\text{H}_5\text{O})_3\text{PO}$                                                       | Solid, M.P. 50° C. <sup>3</sup>  | 245-250° C./5 mm.          | —                | (*)                        | —      |
| $(\text{C}_6\text{H}_5\text{O})_2(2\text{-C}_6\text{H}_5\text{C}_6\text{H}_4\text{O})\text{PO}$   | Liquid <sup>5</sup>              | 250-285° C./5 mm.          | 20               | 6.9                        | 90     |
| $(\text{C}_6\text{H}_5\text{O})_2(2\text{-C}_6\text{H}_5\text{C}_6\text{H}_4\text{O})_2\text{PO}$ | do                               | 273-275° C./0.5 mm.        | —                | —                          | —      |
| $(2\text{-C}_6\text{H}_5\text{C}_6\text{H}_4\text{O})_3\text{PO}$                                 | Solid, M.P. 114° C. <sup>6</sup> | —                          | —                | (*)                        | (*)    |
| "P2-B 72" of Example 3                                                                            | Liquid                           | 228-330° C./5 mm.          | 15               | 8.8                        | 127    |
| $(\text{C}_6\text{H}_5\text{O})_3\text{PO}$                                                       | Solid, M.P. 50° C. <sup>3</sup>  | 245-250° C./5 mm.          | —                | (*)                        | —      |
| $(\text{C}_6\text{H}_5\text{O})_2(4\text{-C}_6\text{H}_5\text{C}_6\text{H}_4\text{O})\text{PO}$   | Solid, M.P. 63° C. <sup>7</sup>  | 302-309° C./10 mm.         | —                | (*)                        | —      |
| $(\text{C}_6\text{H}_5\text{O})_2(4\text{-C}_6\text{H}_5\text{C}_6\text{H}_4\text{O})_2\text{PO}$ | Solid, M.P. 89° C. <sup>7</sup>  | ca. 360° C./7 mm.          | —                | (*)                        | —      |
| $(4\text{-C}_6\text{H}_5\text{C}_6\text{H}_4\text{O})_3\text{PO}$                                 | Solid, M.P. 137° C. <sup>7</sup> | —                          | —                | (*)                        | (*)    |
| "P4-B 70" of Example 2                                                                            | Liquid                           | 230-350° C./5 mm.          | 0                | 7.7                        | 97     |

<sup>1</sup> At normal room temperature.

<sup>2</sup> For at least 95% of the material.

<sup>3</sup> Hand and Magoon, U.S.P. 1,866,852.

<sup>4</sup> Kosolapoff, *Organic Phosphorus Compounds*, Wiley, 1950, pp. 263-264.

<sup>5</sup> Bass, U.S.P. 2,033,918.

<sup>6</sup> Britton, U.S.P. 1,858,659.

<sup>7</sup> Britton and Bass, U.S.P. 2,117,291.

<sup>8</sup> Solid.

tent of 67 percent. This product mixture will be referred to hereinafter as "PN 67."

B. For purposes of comparison, the above procedure is repeated except that the relative proportions of the naphthol and phenol are reversed, that is, there is employed 0.16 lb. mole of beta-naphthol and 0.08 lb. mole of phenol. The reaction product, a viscous liquid which solidifies to a low melting solid after some weeks standing at room temperatures, consists roughly of 4 mole percent triphenyl phosphate, 22 mole percent naphthyl diphenyl phosphate, 48 mole percent dinaphthyl phenyl phosphate, and 27 mole percent trinaphthyl phosphate.

The mixtures of Examples 1-3 are remarkably fluid (at normal room temperatures), especially in view of the fact that at least two of the four components in each mixture are normally solid and therefore also inherently viscous. Surprisingly, the liquid mixtures of this invention appear on the whole substantially no less pourable and no more viscous than the most fluid single member, yet they show an extended liquid range and an overall wide boiling range believed to be of advantage for the purposes of this invention as illustrated in the following examples.

Similarly, by the procedure of Example 1, there can

be prepared a variety of multi-component phenyl two-ring-aryl triesters of orthophosphoric acid coming within the scope of this invention. Alternatively, individually prepared esters may be blended to produce representative compositions. For example, Table 2 shows multi-component phosphate mixtures that can be obtained (A) by the method of Example 1, and (B) by blending the various phosphate esters in the proportions indicated. Compositions are in mole percent to the nearest whole number. The phenyl index represents percent phenyl in the composition and, in the case of the compositions under A, also indicates the mole percent phenol in the starting phenolic mixture.

B. The Deposit-Induced Surface Ignition Test was repeated on the same leaded gasoline composition of (A) in which there was also incorporated a triaryl phosphate as identified in Table 3 below. It should be noted that the results at the 0.05 theory level derive from another engine of the same type so that these results may not be fairly compared with those obtained at the indicated higher phosphorus concentrations. However, the results show that at all concentrations the phenyl two-ring-aryl phosphate compositions of this invention are more effective than the commercially used tricresyl phosphate and cresyl diphenyl phosphate. "PN 67" of Example 1A is also shown superior

TABLE 2.—MULTI-COMPONENT PHENYL TWO-RING-ARYL PHOSPHATE MIXTURES OF THIS INVENTION

| Phosphate/Phenyl Index         | A<br>According to the Proc-<br>ess of Example 1—<br>Mole Percent |    |    | B<br>Blended Composi-<br>tions—Mole Percent |    |    |
|--------------------------------|------------------------------------------------------------------|----|----|---------------------------------------------|----|----|
|                                | 60                                                               | 75 | 79 | 67                                          | 70 | 75 |
| $(C_6H_5O)_3PO$                | 22                                                               | 42 | 49 | 20                                          | 35 | 45 |
| $(C_6H_5O)_2(C_6H_7O)PO$       | 43                                                               | 43 | 39 | 42                                          | 42 | 45 |
| $(C_6H_5O)_2(C_6H_5C_6H_4O)PO$ | 29                                                               | 12 | 60 | 23                                          | 35 | 35 |
| $(C_6H_5O)(C_6H_5C_6H_4O)_2PO$ | 6                                                                | 14 | 20 | 5                                           | 20 | 20 |
| $(C_6H_5O)_3PO$                | 6                                                                | 1  | —  | —                                           | —  | —  |
| $(C_6H_5C_6H_4O)_3PO$          | —                                                                | —  | —  | —                                           | —  | —  |

*Example 4*

The effectiveness of the phosphates of this invention to combat surface ignition is shown by means of the Deposit-Induced Surface Ignition Test hereinafter described, involving the use of a single-cylinder CFR engine operated under the following conditions:

|                                     |       |
|-------------------------------------|-------|
| Engine speed, r.p.m.                | 1800  |
| Compression ratio                   | 9.0:1 |
| Spark timing, ° BTC                 | 20    |
| Commutator timing, ° ATC            | 8     |
| Intake air temp., ° F.              | 200   |
| Jacket temp., ° F.                  | 212   |
| Oil temp., ° F.                     | 160   |
| Manifold air press., inches Hg abs. | 20    |
| Fuel-air ratio                      | 0.075 |

To determine the incidence of surface ignition, the engine is allowed 19.5 minutes under the above conditions, then during the next 0.5 minute the manifold air pressure is increased to 30 inches of Hg absolute (to simulate an acceleration) and the occurrence of preignition (before the normal spark ignition in each cycle) is detected electronically by means of ionization probes inserted in the cylinder head. This cyclic procedure is repeated for a total of 40 hours running time and the observed occurrences of deposit-induced surface ignitions are expressed as counts/hour.

A. A reference line for Deposit-Induced Surface Ignition was established at 63 counts per hour by operating in the above test on a leaded aromatic type gasoline having an octane rating of 106.8 by the Research Method and 99.3 by the Motor Method and which was prepared by adding tetraethyl lead (TEL), ethylene dibromide and ethylene dichloride, in amounts providing 3 ml./gal. of the tetraethyl lead, 0.5 theory of bromine and 1.0 theory of chlorine, to a motor gasoline base fuel composed of catalytic-reformed stocks providing 46 volume percent aromatic hydrocarbons, 1 volume percent olefins and 53 volume percent saturated hydrocarbons and having an octane rating of 98.9 by the Research Method and 89.9 by the Motor Method. With the same fuel composition prepared without the halohydrocarbon scavenger components, the incidence of surface ignition was 130 counts per hour.

to the phenyl naphthyl phosphate composition not of this invention, "PN 33" of Example 1B.

TABLE 3.—REDUCING SURFACE IGNITION WITH TRIARYL PHOSPHATES

| Triaryl Phosphate         | Concen-<br>tration,<br>Theory<br>P | Percent Reduction<br>in Surface Ignition |                  |
|---------------------------|------------------------------------|------------------------------------------|------------------|
|                           |                                    | TEL<br>(mm.) <sup>1</sup>                | TEL <sup>2</sup> |
| "PN 67" of Example 1A     | 0.05                               | 85                                       | —                |
| "P4-B 70" of Example 2    | 0.05                               | 80                                       | —                |
| Tricresyl phosphate       | 0.05                               | 35                                       | —                |
| "PN 67" of Example 1A     | 0.1                                | 57                                       | —                |
| "P2-B 72" of Example 3    | 0.1                                | 50                                       | 52               |
| Cresyl diphenyl phosphate | 0.1                                | 24                                       | 28               |
| "PN 67" of Example 1A     | 0.2                                | 79                                       | —                |
| "PN 33" of Example 1B     | 0.2                                | 69                                       | —                |
| Tricresyl phosphate       | 0.2                                | 62                                       | —                |

<sup>1</sup> Halohydrocarbon scavengers present in the proportions as described above in A.

<sup>2</sup> No halohydrocarbon scavenger present.

It will be noted that the above demonstrated superiority of the phosphate compositions of this invention to control surface ignition is based on the use in an aromatic type gasoline. In contrast, "PN 67" of Example 1A is less effective in this regard than tricresyl phosphate when employed in a non-aromatic gasoline. For example, 4 ml./gal. of tetraethyl lead, 1 theory of bromine as ethylene dibromide and either 0.0 or 0.2 theory of phosphorus as triaryl phosphate was blended into a base fuel which consisted of 5.5 volume percent aromatics, 20 volume percent olefins and 92.5 volume percent saturates (thereby raising the Research Method octane rating from 93 to 106 and the Motor Method rating from 90 to 103). According to the Deposit-Induced Ignition Test, the phenyl naphthyl phosphate composition "PN 67" caused a 27% reduction, the tricresyl phosphate a 43% reduction, in the surface ignition rate.

The phenyl two-ring-aryl phosphates of this invention are also superior to commercial prior art triaryl phosphate additives when employed in aromatic type motor gasoline in high compression multicylinder automotive engines, as shown in the following example.

*Example 5*

Tetraethyl lead, ethylene dichloride and ethylene dibromide, with and without a triaryl phosphate as described

below, were blended into the gasoline base stock described in Example 4A in amounts providing 4.28 grams/gal. of lead, 1.0 theory of chlorine, 0.5 theory of bromine and 0.0, 0.3 or 0.7 theory of phosphorus as identified below. The resulting fuels (having Research Method octane ratings of about 107.8 and Motor Method ratings of about 100.4) were employed in the operation of a 12.5:1 compression ratio GM Research eight cylinder engine under medium-duty, cyclic conditions involving 3.3 minutes at 1850 r.p.m. and 25 B.H.P. deceleration under load to idle, 1 minute idle at 700 r.p.m., and acceleration under load, with one of twelve accelerations per hour at full-throttle and eleven of twelve per hour part-throttle. The incidence of surface ignition occurring during the period of acceleration at full-throttle was sensed by means of ionization probes in each cylinder head. The results are tabulated in Table 4 as counts/hour (observed as a steady value over a period of at least 100 consecutive hours of operation) and percent lowering of preignition effected by the additives.

TABLE 4.—REDUCING SURFACE IGNITION IN MULTICYLINDER ENGINE TEST WITH TRIARYL PHOSPHATES

| Triaryl Phosphate         | Conc. of P, Theory | Total Test Time, Hours | Pre-ignition Counts/Hr. | Reduction in Pre-ignition, Percent |
|---------------------------|--------------------|------------------------|-------------------------|------------------------------------|
| None                      |                    | 235                    | 84                      | 0                                  |
| "PN 67" of Example 1A     | 0.3                | 185                    | 14                      | 83                                 |
| Cresyl diphenyl phosphate | 0.3                | 165                    | 26                      | 69                                 |
| Cresyl diphenyl phosphate | 0.7                | 215                    | 14                      | 83                                 |

It will be noted that a much higher dosage of the commercial cresyl diphenyl phosphate (0.7 theory P) is needed to match the effectiveness of the phenyl naphthyl phosphate composition "PN 67" of this invention at the 0.3 theory P level.

At the end of each run, the intake system was found clean and free of abnormal deposits. In general, combustion chamber deposits tended to be lower with phosphorus present in the fuel, and both visual inspection and compression pressure tests showed no adverse effect of phosphorus on the valves. Also, it was observed (in the single cylinder as well as the multicylinder engine tests) that, while none of the phosphates had a significantly adverse effect on engine octane requirement, in general the lower the surface ignition count the lower the engine octane requirement.

#### Example 6

The phosphate compositions of this invention are also highly effective to combat spark plug misfiring, as illustrated in the Spark Plug Misfiring Test described below, involving the operation of a standard production V-8 Oldsmobile engine according to a spark plug deposit accumulation cycle and a Spark Plug Rating Cycle.

In the deposit accumulation cycle, new AC-44 plugs are installed in a clean engine and the engine run for a total of 20 or more hours under the following conditions:

| Time Secs. | Speed | Load           | Oil Temp., °F. | Coolant Temp. in °F. | Coolant Temp. out °F. |
|------------|-------|----------------|----------------|----------------------|-----------------------|
| 30         | 500   | 0              | 160            | 145                  | 160                   |
| 30         | 1,500 | Road (15 H.P.) | ±3             | ±3                   | ±3                    |

Production engine adjustments are maintained during the entire test. At 20 hour intervals, the plugs are removed from the engine, rated (as below) and returned for an additional 20 hours accumulation of deposits. This is repeated until the total number of allotted test hours has elapsed or until a particular level of plug performance is observed in the rating procedure.

In the Spark Plug Rating Cycle, each of the above ex-

posed plugs is rated individually in the No. 1 cylinder of the engine. But first, new plugs are installed in all cylinders and the engine load adjusted to give 3200 r.p.m. at the end of a 20 second wide-open-throttle (WOT) acceleration from 1500 r.p.m., 30 H.P. load. The WOT acceleration is repeated several times to bring the engine to equilibrium. Then the test plug is installed and the engine is given (a) a warmup of 2 minutes alternating between 800 r.p.m. no load (idle) and 1500 r.p.m. brake horsepower (road load) then (b) one full-throttle acceleration during which spark plug misfire is detected by means of an ion gap counter.

By means of this test, various triaryl phosphates were compared as to effectiveness as spark plug antifoulants in a typical leaded aromatic type motor gasoline—the fuel more particularly described in Example 4A. The results are expressed in Table 5 in terms of the number of hours of plug exposure to 10% misfiring. Such time, which is not a multiple of 20 hours, is obtained by interpolation.

TABLE 5.—EFFECTIVENESS OF TRIARYL PHOSPHATES AS SPARK PLUG ANTIFOULANTS

| Triaryl phosphate:            | Plug performance hrs. to 10% misfire |
|-------------------------------|--------------------------------------|
| None                          | 46                                   |
| Cresyl diphenyl phosphate     | 73                                   |
| 2-biphenyl diphenyl phosphate | 84                                   |
| "P2-B 72" of Example 3        | 99                                   |
| "PN 67" of Example 1          | >100                                 |

It will be noted that the 2-biphenyl diphenyl phosphate is closely similar in its empirical constitution (phenyl content=67%) to "P2-B 72" (phenyl content=72%) and that these two compositions and "PN 67" as well are all roughly comparable in fluidity characteristics (Table 1 above), yet the wide-boiling multi-component compositions of this invention appear significantly more effective in this spark plug test than the single compounds.

#### Example 7

To a full boiling gasoline (initial point 100° F., 10% point 132° F., 50% point 222° F., 90% point 323° F. and end point 398° F.) a blend consisting essentially of 55% reformat, 30% alkylate and 15% isopentane, and

composed of 28% aromatics, 1% olefins and 71% saturates all by volume, was added 3 ml. tetraethyl lead per gallon, 1.0 theory of ethylene dichloride, 0.5 theory of ethylene dibromide, and 0.4 or 1.0 theory P (th. P) as identified below in Table 6. The antiknock properties, Research octane number (R.O.N.) of the fuel compositions were determined by the ASTM Research Method 75 with the results shown in Table 6.

TABLE 6.—EFFECT OF TRIARYL PHOSPHATE ON LEADED RESEARCH OCTANE NUMBER

| Phosphate                 | (0.4 th. P)<br>Series 1,<br>R.O.N. | (1.0 th. P)<br>Series 2,<br>R.O.N. |
|---------------------------|------------------------------------|------------------------------------|
| None                      | 101.4                              | 102.2                              |
| Cresyl diphenyl phosphate | 101.4                              | 102.0                              |
| "PN 67" of Example 1      | 101.4                              | 102.0                              |
| "P4-B 70" of Example 2    | 101.4                              | 101.8                              |
| P2-B 72" of Example 3     | 101.4                              | 101.8                              |

5

TABLE 7.—EFFECT OF TRIARYL PHOSPHATES ON CARBURETOR ICING OF MOTOR GASOLINE

| Triaryl Phosphate             | Concentration |          | Minutes of Stall-Free Operation |
|-------------------------------|---------------|----------|---------------------------------|
|                               | G./gal.       | Theory P |                                 |
| "PN 67" of Example 1          | 0.38          | 0.1      | 1.5                             |
| 2-Naphthyl diphenyl phosphate | 0.38          | 0.1      | 2.0                             |
|                               | 1.15          | 0.3      | 0.5                             |
|                               | 1.15          | 0.3      | 0.5                             |
| None                          | 0             | 0        | 0.5                             |

15

The tabulated data show that the triaryl phosphates of this invention are substantially non-antagonistic to tetraalkyl lead antiknocks.

Phosphate compositions of this invention, exemplified by "PN 67" of Example 1A, provide still another benefit of inhibiting engine stalling due to carburetor icing—a common occurrence in the operation of an internal combustion engine, during warm-up and idling, under cool, humid atmospheric conditions. Stalling is attributed to the formation of ice particles in the carburetor, especially on the throttle plate and surrounding walls, caused by a lowering in the temperature of the metal parts of the carburetor as the fuel vaporizes.

#### Example 8

Antistalling effectiveness of the additives of this invention is illustrated by means of the Carburetor Icing Test described below which is designed to evaluate carburetor icing tendencies of motor gasolines and the effectiveness of additives under severe icing conditions. The engine is a standard 6-cylinder Chevrolet engine, having a horsepower rating of 86 at 3400 r.p.m. and a displacement of 216.5 cu. in., operated under the following conditions:

|                          |                |
|--------------------------|----------------|
| Intake air               | 38-40° F.      |
| Relative humidity        | Approx. 100%.  |
| Engine load              | 10 horsepower. |
| Engine speed             | 1500 r.p.m.    |
| Idle speed               | 350-400 r.p.m. |
| Fuel temp. to carburetor | 50-55° F.      |

Before starting each run, the throttle plate is first cleaned and conditioned by soaking it in alcohol for 0.5 minute at a temperature of 40° F. Fuels are rated by the number of minutes of open-throttle operation at 1500 r.p.m. under a load necessary to cause stalling while idling. With commercial gasolines without antiicing protection, stalling generally occurs within 0.5 to 1.25 minutes. The base gasoline used in this series of tests has the following characteristics:

|                           |      |
|---------------------------|------|
| Gravity, ° API            | 64.7 |
| Reid vapor press., p.s.i. | 13.2 |
| ASTM distn., ° F.:        |      |
| IBP                       | 76   |
| 10%                       | 104  |
| 50%                       | 201  |
| 90%                       | 332  |
| EP                        | 407  |
| Aromatic, vol. percent    | 25   |
| Olefins                   | 12.2 |
| Saturates                 | 62.8 |

70

The results obtained with this gasoline are given in Table 7 and show that the phosphate compositions of this invention also provide significant antistall resistance to motor fuels normally tending to stall due to carburetor icing.

75

TABLE 8.—MULTIPURPOSE ANTISTALL AND ANTI-PREIGNITION PHOSPHORUS COMPOSITIONS

| Ingredient                              | Percent Weight |      |
|-----------------------------------------|----------------|------|
|                                         | A              | B    |
| Alkylamine salt of alkyl acid phosphate | 13.7           | 8.0  |
| Methanol                                | 33.4           | 59.1 |
| Kerosene                                |                | 2.0  |
| "P2-B 72" of Example 3                  | 53.9           | 30.9 |

Tetraethyl lead antiknock blends A and B of Table 9 below, having improved deposit-modifier characteristics, were prepared by mixing 1.20 and 28.8 parts of "PN 67" of Example 1A with 100 parts of a mixture of the other ingredients shown in Table 9 to form clear, homogeneous liquid blends.

TABLE 9.—ANTIKNOCK BLENDS OF THIS INVENTION

| Ingredient                | Parts by Weight | Scavenger Theories per Atom of Pb |     |
|---------------------------|-----------------|-----------------------------------|-----|
|                           |                 | A                                 | B   |
| Tetraethyl lead.....      | 61.5            |                                   |     |
| Ethylene dichloride.....  | 18.8            | 1.0                               | 1.0 |
| Ethylene dibromide.....   | 17.9            | 0.5                               | 0.5 |
| Kerosene (inerts).....    | 1.8             |                                   |     |
| Orange dye.....           | 0.05            |                                   |     |
| "PN 67" of Example 1..... | 1.2; 28.8       | 0.025                             | 0.6 |

Similar mixes can be prepared from the other phosphate mixtures of this invention, by substituting for example "P4-B 70" of Example 2 and "P2-B 72" of Example 3.

In addition to those described in the foregoing examples, a wide variety of improved motor gasolines can be formulated in accordance with this invention. For example multi-component phosphate composition of phenyl index 60 described in Table 2 can be blended to a concentration of 0.39 gram/gal. (about 0.1 theory) with a motor gasoline characterized by its composition by volume of 24 percent of aromatics, 42 percent of olefins, and 34 percent of saturates, its content of 5.07 ml./gal. of tetraethyl lead antiknock mix comprising 3 ml./gal. of tetraethyl lead, 1.5 grams/gal. of ethylene dichloride (1 theory), and 1.44 grams/gal. of ethylene dibromide (0.5 theory), and the base fuel's API gravity of 64.1° (according to ASTM Test Procedure D-287), vapor pressure of 13.8 p.s.i. (according to ASTM Test Procedure D-323) and (according to ASTM Test Procedure D-86) initial boiling point of 84° F., 10 percent point of 110° F., mid-boiling point of 195° F., 90 percent point of 306° F., and final boiling point of 387° F.

Similarly there can be prepared a motor fuel containing 3.18 grams Pb./gal. as tetraethyl lead with conventional scavengers (1 theory ethylene dichloride and 0.5 theory ethylene dibromide) and 0.3 theory of phosphorus by blending the tetraethyl lead, the scavengers, and the Table 2 composition of phenyl index 79 into a gasoline base stock composed by volume of 44 percent of aromatics, 17 percent of olefins, and 39 percent of saturates, and having a gravity of 54.7° API, a vapor pressure of 9.6 p.s.i., an initial boiling point of 97° F., a 10 percent point of 129° F., a mid-boiling point of 234° F., a 90 percent point of 307° F., and final boiling point of 350° F.

Similarly, also, three finished fuels can be prepared from a base stock containing by volume 24 percent aromatics, 2 percent olefins, 74 percent saturates and having a gravity of 61.5° API, a vapor pressure of 9.5 p.s.i., initial boiling point of 88° F., a 10 percent point of 130° F., mid-boiling point of 222° F., a 90 percent point of 318° F., and final boiling point of 384° F., (a) by blending one portion of this base fuel with 2 grams Pb./gal. as tetramethyl lead, 0.025 theory of P as the composition of phenyl index 67 described in Table 2, 1.0 theory ethylene dichloride and 0.5 theory ethylene dibromide; (b) by blending a second portion with 0.2 theory of P as "P2-B 72" of Example 3 and 4.0 grams Pb./gal. in the form of a mixture of tetraalkyl leads analyzing approximately 6 mole percent tetramethyl lead, 25 mole percent trimethyl ethyl lead, 38 mole percent dimethyl diethyl lead, and 25 mole percent methyltriethyl lead, and 6 mole percent tetraethyl lead, together with 0.5 theory bromine as ethylene dibromide and 1.0 theory chlorine as ethylene dichloride;

and (c) by blending the third portion of the base stock with 0.1 theory of P as the composition having phenyl index 75 in Table 2 and 3.25 grams Pb./gal. as an equimolar mixture of tetramethyl lead and tetraethyl lead and containing conventional scavenging agents as in the second portion.

Still another useful leaded and phosphated fuel composition of this invention can be obtained by adding "PN 67" of Example 1A at a concentration of 2.31 grams/gal. (0.6 theory) to a motor gasoline composed by volume 15 percent aromatics, 16 percent olefins, and 69 percent saturates and containing 3.0 grams Pb./gal. as tetraethyl lead together with 1.5 theories ethylene dichloride as scavenging agent.

It will be understood that the preceding examples have been given for illustrative purposes solely and that this invention is not limited to the specific embodiments described therein. On the other hand, it will be readily apparent to those skilled in the art that, subject to the limitations set forth in the general description, variations and modifications can be made in the materials, proportions and techniques employed without departing from the spirit or scope of this invention.

From the foregoing description, it will be apparent that this invention provides novel triaryl phosphate compositions, novel antiknock blends containing them, and novel motor fuels composed of aromatic base fuels containing organolead antiknock agents and the triaryl phosphate compositions. The triaryl phosphate compositions of this invention have a novel combination of advantageous properties, whereby, when they are used in such motor fuels, they serve a multiplicity of purposes to impart to the motor fuels a combination of highly beneficial properties not heretofore obtainable with a single additive or with related phosphate compositions. Accordingly, it will be apparent that this invention constitutes a valuable advance in and contribution to the art.

The embodiments of the invention in which an exclusive property or privilege is claimed are defined as follows:

1. A triaryl phosphate composition consisting essentially of a mixture of
  - about 20 to about 50 mole percent of triphenyl phosphate,
  - about 35 to about 60 mole percent of a two-ring-aryl diphenyl phosphate,
  - about 10 to about 30 mole percent of a di(two-ring-aryl) phenyl phosphate, and
  - 0 to about 6 mole percent of a tri(two-ring-aryl) phosphate,
  - the mixed phosphates of (b) and (c) constituting a total of about 50 to about 80 mole percent of said mixture, and
  - the phenyl groups constituting about 60 to about 80 mole percent of all aryl groups in said phosphates.
2. A triaryl phosphate composition consisting essentially of a mixture of
  - about 25 to about 45 mole percent of triphenyl phosphate,
  - about 40 to about 55 mole percent of a two-ring-aryl diphenyl phosphate, and
  - about 15 to about 25 mole percent of a di(two-ring-aryl) phenyl phosphate,
  - the mixed phosphates of (b) and (c) constituting a total of about 55 to about 75 mole percent of said mixture, and
  - the phenyl groups constituting about 65 to about 75 mole percent of all aryl groups in said phosphates.
3. A triaryl phosphate composition consisting essentially of a mixture of
  - about 20 to about 50 mole percent of triphenyl phosphate,
  - about 35 to about 60 mole percent of a naphthyl diphenyl phosphate,

- (c) about 10 to about 30 mole percent of a dinaphthyl phenyl phosphate, and
  - (d) 0 to about 6 mole percent of a trinaphthyl phosphate,
  - (e) the mixed phosphates of (b) and (c) constituting a total of about 50 to about 80 mole percent of said mixture, and
  - (f) the phenyl groups constituting about 60 to about 80 mole percent of all aryl groups in said phosphates.
4. A triaryl phosphate composition consisting essentially of a mixture of
- (a) about 28 to about 32 mole percent of triphenyl phosphate,
  - (b) about 44 to about 48 mole percent of a naphthyl diphenyl phosphate,
  - (c) about 20 to about 24 mole percent of a dinaphthyl phenyl phosphate, and
  - (d) 0 to about 4 mole percent of a trinaphthyl phosphate.
5. A triaryl phosphate composition consisting essentially of a mixture of
- (a) about 20 to about 50 mole percent of triphenyl phosphate,
  - (b) about 35 to about 60 mole percent of a biphenyl diphenyl phosphate,
  - (c) about 10 to about 30 mole percent of a di-biphenyl phenyl phosphate, and
  - (d) 0 to about 6 mole percent of a tri-biphenyl phosphate,
  - (e) the mixed phosphates of (b) and (c) constituting a total of about 50 to about 80 mole percent of said mixture, and
  - (f) the phenyl groups constituting about 60 to about 80 mole percent of all aryl groups in said phosphates.
6. A triaryl phosphate composition consisting essentially of a mixture of
- (a) about 29 to about 33 mole percent of triphenyl phosphate,
  - (b) about 51 to about 55 mole percent of a biphenyl diphenyl phosphate,
  - (c) about 12 to about 16 mole percent of a di-biphenyl phenyl phosphate, and
  - (d) 0 to about 4 mole percent of a tri-biphenyl phosphate.
7. An antiknock blend consisting essentially of
- (A) an organolead antiknock agent,
  - (B) at least one halohydrocarbon scavenger for lead in an amount providing 1 to 5 atoms of halogen of atomic numbers 17-35 for each atom of lead of said organolead antiknock agent, and
  - (C) a triaryl phosphate composition as defined in claim 1 in an amount providing about 0.013 to about 0.4 atom of phosphorus for each atom of lead of said organolead antiknock agent.
8. An antiknock blend consisting essentially of
- (A) a tetraalkyl lead antiknock agent, in which the alkyl groups contain 1-2 carbon atoms,
  - (B) at least one ethylene dihalide in which the halogens are of atomic numbers 17-35 in an amount to provide about 2 to about 3 atoms of halogen and not more than 2 atoms of bromine for each atom of lead of said tetraalkyl lead antiknock agent, and
  - (C) a triaryl phosphate composition as defined in claim 1 in an amount providing about 0.013 to about 0.4 atom of phosphorus for each atom of lead of said tetraalkyl lead antiknock agent.
9. An antiknock blend consisting essentially of
- (A) a tetraalkyl lead antiknock agent, in which the alkyl groups contain 1-2 carbon atoms,
  - (B) at least one ethylene dihalide in which the halogens are of atomic numbers 17-35 in an amount to provide about 2 to about 3 atoms of halogen and not more than 2 atoms of bromine for each atom of lead of said tetraalkyl lead antiknock agent, and

- (C) a triaryl phosphate composition as defined in claim 3 in an amount providing about 0.013 to about 0.4 atom of phosphorus for each atom of lead of said tetraalkyl lead antiknock agent.
10. An antiknock blend consisting essentially of
- (A) a tetraalkyl lead antiknock agent, in which the alkyl groups contain 1-2 carbon atoms,
  - (B) at least one ethylene dihalide in which the halogens are of atomic numbers 17-35 in an amount to provide about 2 to about 3 atoms of halogen and not more than 2 atoms of bromine for each atom of lead of said tetraalkyl lead antiknock agent, and
  - (C) a triaryl phosphate composition as defined in claim 4 in an amount providing about 0.013 to about 0.4 atom of phosphorus for each atom of lead of said tetraalkyl lead antiknock agent.
11. An antiknock blend consisting essentially of
- (A) a tetraalkyl lead antiknock agent, in which the alkyl groups contain 1-2 carbon atoms,
  - (B) at least one ethylene dihalide in which the halogens are of atomic numbers 17-35 in an amount to provide about 2 to about 3 atoms of halogen and not more than 2 atoms of bromine for each atom of lead of said tetraalkyl lead antiknock agent, and
  - (C) a triaryl phosphate composition as defined in claim 5 in an amount providing about 0.013 to about 0.4 atom of phosphorus for each atom of lead of said tetraalkyl lead antiknock agent.
12. An antiknock blend consisting essentially of
- (A) a tetraalkyl lead antiknock agent, in which the alkyl groups contain 1-2 carbon atoms,
  - (B) at least one ethylene dihalide in which the halogens are of atomic numbers 17-35 in an amount to provide about 2 to about 3 atoms of halogen and not more than 2 atoms of bromine for each atom of lead of said tetraalkyl lead antiknock agent, and
  - (C) a triaryl phosphate composition as defined in claim 6 in an amount providing about 0.013 to about 0.4 atom of phosphorus for each atom of lead of said tetraalkyl lead antiknock agent.
13. A motor fuel consisting essentially of a mixture of liquid hydrocarbons boiling in the gasoline boiling range of which at least 15% by volume are aromatic hydrocarbons of the character of those occurring in catalytically cracked and reformed gasolines, said mixture of hydrocarbons having an octane rating of at least 80 as measured by the ASTM Research Method, and which motor fuel contains
- (A) an organolead antiknock agent in an amount to provide 0.1 to about 6 grams of lead for each gallon of the motor fuel,
  - (B) at least one halohydrocarbon scavenger for lead in an amount providing 1 to 5 atoms of halogen of atomic numbers 17-35 for each atom of lead of said organolead antiknock agent, and
  - (C) a triaryl phosphate composition as defined in claim 1 in an amount providing about 0.013 to about 0.4 atom of phosphorus for each atom of lead of said organolead antiknock agent.
14. A motor fuel consisting essentially of a mixture of liquid hydrocarbons boiling in the gasoline boiling range of which at least 15% by volume are aromatic hydrocarbons of the character of those occurring in catalytically cracked and reformed gasolines, said mixture of hydrocarbons having an octane rating of at least 80 as measured by the ASTM Research Method, and which motor fuel contains
- (A) a tetraalkyl lead antiknock agent in which the alkyl groups contain 1 to 2 carbon atoms in an amount to provide 0.1 to about 6 grams of lead for each gallon of the motor fuel,
  - (B) at least one halohydrocarbon scavenger for lead in an amount providing 1 to 5 atoms of halogen of atomic numbers 17-35 for each atom of lead of said tetraalkyl lead antiknock agent, and

(C) a triaryl phosphate composition as defined in claim 1 in an amount providing about 0.013 to about 0.4 atom of phosphorus for each atom of lead of said tetraalkyl lead antiknock agent.

15. A motor fuel consisting essentially of a mixture of liquid hydrocarbons boiling in the gasoline boiling range of which at least 15% by volume are aromatic hydrocarbons of the character of those occurring in catalytically cracked and reformed gasolines, said mixture of hydrocarbons having an octane rating of at least 85 as measured by the ASTM Research Method, and which motor fuel contains

- (A) a tetraalkyl lead antiknock agent in which the alkyl groups contain 1 to 2 carbon atoms in an amount to provide 0.1 to about 6 grams of lead for each gallon of the motor fuel,
- (B) at least one halohydrocarbon scavenger for lead in an amount providing about 2 to about 3 atoms of

halogen of atomic numbers 17-35 for each atom of lead of said tetraalkyl lead antiknock agent, and

(C) a triaryl phosphate composition as defined in claim 1 in an amount providing about 0.013 to about 0.4 atom of phosphorus for each atom of lead of said tetraalkyl lead antiknock agent.

## References Cited

## UNITED STATES PATENTS

|    |           |         |                |       |       |
|----|-----------|---------|----------------|-------|-------|
| 10 | 2,862,801 | 12/1958 | DeWitt         | ----- | 44-69 |
|    | 2,999,739 | 9/1961  | Heron          | ----- | 44-69 |
|    | 3,038,791 | 6/1962  | Orloff et al.  | ----- | 44-69 |
|    | 3,052,528 | 9/1962  | Roddick et al. | ----- | 44-69 |

## FOREIGN PATENTS

683,405 11/1952 Great Britain.

DANIEL E. WYMAN, Primary Examiner.

W. J. SHINE, Assistant Examiner.